

Nov. 22, 1966

SATORU TAGUCHI ETAL 3,287,183

PROCESS FOR PRODUCING SINGLE-ORIENTED SILICON  
STEEL SHEETS HAVING A HIGH MAGNETIC INDUCTION  
Filed June 22, 1964

7 Sheets-Sheet 1

FIG. 1



INVENTORS.

Satoru Taguchi

Akira Sakakura

Hironori Takashima

BY *Wenderoth, Lind*  
*and Boxach*  
*Attorneys*

Nov. 22, 1966

SATORU TAGUCHI ETAL 3,287,183

PROCESS FOR PRODUCING SINGLE-ORIENTED SILICON  
STEEL SHEETS HAVING A HIGH MAGNETIC INDUCTION

Filed June 22, 1964

7 Sheets-Sheet 2

FIG. 2



Nov. 22, 1966

SATORU TAGUCHI ET AL 3,287,183

PROCESS FOR PRODUCING SINGLE-ORIENTED SILICON  
STEEL SHEETS HAVING A HIGH MAGNETIC INDUCTION

Filed June 22, 1964

7 Sheets-Sheet 3

FIG. 3



| Reduction rate of first cold-rolling step (%) | 0                                    | 10   | 20   | 30   | 40   | 50   | 60   | 70   | 80   |      |
|-----------------------------------------------|--------------------------------------|------|------|------|------|------|------|------|------|------|
| Reduction rate of final cold-rolling step (%) | Thickness of hot-rolled sheet 7.0 mm | 95.6 | 95.1 | 94.5 | 93.7 | 92.7 | 91.2 | 89.0 | 85.3 | 78.0 |
| 5.0                                           | 94.0                                 | 93.3 | 92.5 | 91.4 | 90.0 | 88.0 | 85.0 | 80.0 | 70.0 |      |
| 3.4                                           | 91.2                                 | 90.2 | 89.0 | 87.4 | 85.3 | 82.4 | 78.0 | 70.7 | 56.0 |      |
| 3.0                                           | 90.0                                 | 88.9 | 87.5 | 85.7 | 83.3 | 80.0 | 75.0 | 66.7 | 50.0 |      |
| 2.6                                           | 88.5                                 | 87.2 | 85.6 | 83.6 | 80.9 | 77.0 | 71.2 | 61.7 | 42.5 |      |
| 1.8                                           | 83.3                                 | 81.4 | 79.1 | 76.1 | 72.2 | 66.4 | 58.2 | 44.3 | 16.5 |      |

INVENTORS.

Satoru Taguchi

Akira Sakakura

Hironori Takashima

BY Wenderoth, Hind  
and Paack

Attorneys

Nov. 22, 1966

SATORU TAGUCHI ET AL.

3,287,183

PROCESS FOR PRODUCING SINGLE-ORIENTED SILICON STEEL SHEETS HAVING A HIGH MAGNETIC INDUCTION  
Filed June 22, 1964 7 Sheets

7 Sheets-Sheet 4

FIG. 4 (1)



FIG. 5 (1)



*INVENTORS.*

Satoru Taguchi

Akira Sakakura

Hironori Takashima

BY Wenderoth, Lind  
and Ponack

attorneys

Nov. 22, 1966

SATORU TAGUCHI ET AL.

3,287,183

PROCESS FOR PRODUCING SINGLE-ORIENTED SILICON STEEL SHEETS HAVING A HIGH MAGNETIC INDUCTION

Filed June 22, 1964

7 Sheets-Sheet 5

FIG. 4 (2)



FIG. 5 (2)



*INVENTORS.*

Satoru Taguchi

Akira Sakakura

Hironori Takashima

BY WENDROTH, Lind  
and Panack

Attorneys

Nov. 22, 1966

SATORU TAGUCHI ET AL.

3,287,183

PROCESS FOR PRODUCING SINGLE-ORIENTED SILICON STEEL SHEETS HAVING A HIGH MAGNETIC INDUCTION

31  
Filed June 22, 1964

7 Sheets-Sheet 6

FIG. 4 (3)



FIG. 5 (3)



*INVENTORS,*

Satoru Taguchi

Akira Sakakura

Hironori Takashima

BY WENDEROTH, Lind  
and Ponack

Attorneys

Nov. 22, 1966

SATORU TAGUCHI ETAL

3,287,183

PROCESS FOR PRODUCING SINGLE-ORIENTED SILICON  
STEEL SHEETS HAVING A HIGH MAGNETIC INDUCTION

Filed June 22, 1964

7 Sheets-Sheet 7

FIG. 6



Annealing temperature (°C)  
before final cold-rolling

INVENTORS.

Satoru Taguchi

Akira Sakakura

Hironori Takashima

BY *Wenderoth, Lind  
and Posack*  
*Attorneys*

3,287,183

## PROCESS FOR PRODUCING SINGLE-ORIENTED SILICON STEEL SHEETS HAVING A HIGH MAGNETIC INDUCTION

Satoru Taguchi, Akira Sakakura, and Hironori Takashima, Kitakyushu, Fukuoka, Japan, assignors to Yawata Iron & Steel Co., Ltd., Tokyo, Japan, a corporation of Japan

Filed June 22, 1964, Ser. No. 376,627  
4 Claims. (Cl. 148—111)

This invention relates to processes for producing silicon steel sheets and more particularly to a process for producing single-oriented silicon steel sheets having a high magnetic induction.

Single-oriented silicon steel sheets are to be used mostly as iron cores for transformers and other electric devices. For their magnetic characteristics, excitation characteristics (the relation between the intensity of the magnetic field and the magnetic induction) and core loss characteristics (the relation between the magnetic induction and the core loss value) must be favorable. The excitation characteristics are determined depending on the magnitude of the magnetic induction induced in the iron core by the given intensity of the magnetic field. For example, the magnetic induction generated in the iron core by the intensity  $H=10$  (Oe) of the magnetic field is represented as  $B_{10}$ . With the iron core high in  $B_{10}$ , a small ampere turn will do to generate the same magnetic induction and therefore the electric device can be made small.

The core loss is an energy loss lost from the iron core in case a prescribed alternating current magnetic induction is given to the iron core. Therefore, the core loss should be as small as possible. In the case of single-oriented silicon steel sheets, the core loss in the case of 50 cycles and an alternating current magnetic induction of 15,000 gauss is represented with  $W 15/50$ .

More than about 70% of the cost of production of a transformer is said to be the material cost. It is therefore advisable to reduce the material cost by making the transformer as small as possible.

Generally, in order to reduce the weight of the iron core of an electric device, the iron core must be used in a place where the magnetic induction is high. However, a large exciting electric power will be required therefor, thus the exciting electric power will become larger than the advantage obtained by the reduction of the weight of the iron core and the problem caused thereby will be larger.

Further, if the iron core is used in a place where the magnetic induction is high, the core loss value will quickly increase and the increase of the core loss caused by using the iron core in the place where the magnetic induction is high will be larger than the decrease of the core loss by the reduction of the weight of the core. Therefore, today, unless an iron core material excellent in excitation characteristics (high in the value of  $B_{10}$ ) can be produced, the weight reduction and therefore the material cost reduction of an electric device will not be able to be expected. Consequently, the supply of single-oriented silicon steel sheets high in  $B_{10}$  is strongly desired by electric manufacturers.

Now, in order to improve the magnetic property of a single-oriented silicon steel sheet, it is necessary first to highly arrange in the rolling direction the  $\langle 100 \rangle$  axis of the crystal grains forming the steel sheet and second to reduce the impurities in the final product to be as little as possible.

Since a process for producing single-oriented silicon steel sheets by two-step rolling was invented by N. P. Goss, numerous improvements and suggestions have been made and the magnetic induction and core loss value have

been improved year after year. In recent years, due to the development of steel making, surface treating and annealing techniques, the core loss value has become considerably lower. However, the improvement of the magnetic induction  $B_{10}$  may be said to be in a saturated state. Even the so far reported highest value is, as shown in U.S. Patent No. 2,867,557,  $B_{10}=18,690$  gauss at the maximum, ranging from 17,610 to 18,690 gauss and averaging 18,090 gauss.

10 An object of the present invention is to provide a product far superior in magnetic characteristics to any conventional single-oriented silicon steel sheet.

Another object of the present invention is to provide a process for producing single-oriented silicon steel sheets 15 of a high magnetic induction showing  $B_{10}$  of at least 18,000 gauss and 19,100 gauss at the maximum.

Other objects of the present invention and the substance of the invention will be able to be more completely understood with reference to the following specification and claims together with the accompanying drawings in which:

FIGURE 1 is a diagram showing excitation effective volt-ampere curves of a typical product A of the present invention and a typical product B of a conventional 25 single-oriented silicon steel sheet;

FIGURE 2 is a diagram showing a relation between the content of acid-soluble Al and S in an ingot and the magnetic induction  $B_{10}$  in the rolling direction of the product;

FIGURE 3 is a diagram showing a relation between 30 the combination of cold-rolling reduction in thickness and the magnetic induction  $B_{10}$  in the rolling direction of the product;

FIGURE 4 shows (110) pole FIGURES 1 and 2 and a (100) pole FIGURE 3 showing the crystal orientation 35 after each annealing step in case a product is obtained in the typical treating step of the present invention;

FIGURE 5 shows (110) pole FIGURES 1 and 2 and a (100) pole FIGURE 3 showing the crystal orientation after each annealing step in case a product is obtained 40 in a conventional typical treating step for producing single-oriented silicon steel sheets;

FIGURE 6 is a diagram showing a relation between the temperature of annealing carried out just before the final cold-rolling step and the magnetic induction  $B_{10}$  in 45 the rolling direction of the product.

According to the present invention, a silicon steel material of specified contents of such elements as C, S and acid-soluble Al is hot-rolled to be a hot-rolled sheet, which is further subjected to special cold-rolling and annealing 50 different from conventional ones to be a product. That is to say, in the process, the thickness of the final product is obtained by at least more than one annealing step and at least one or more cold-rolling steps. Especially there is a feature that the reduction in thickness in the final cold-rolling is so high as to be in the range of 81 to 95% and that the reduction in thickness in other cold-rolling steps 55 than the final cold-rolling step is kept to be in the range of 5 to 40%. The two annealing steps to be carried out after the final cold-rolling, that is, the annealing at such low temperature as 750 to 850° C. to give a primary recrystallization texture to a steel sheet and to decarburize it and the annealing at such high temperature as above 1000° C. for a long time to produce expected secondary recrystallization grains of the (110)[001] orientation 60 may be carried out in the same manner as in the generally known art. To be specified in the annealing step in the present invention is the annealing condition before the final cold-rolling (the final intermediate annealing condition). That is to say, before this annealing is carried out, the steel sheet must contain 0.020 to 0.080% C. and the annealing should be carried out at such high temperature as 950 to 1200° C. After this annealing, AlN must be 65

formed in the steel sheet, and the content of AlN must be such that N as AlN (N bound in the form of AlN) is more than 0.0020%.

By treating the hot-rolled sheet of such composition as has been described above by cold-rolling and annealing conditions quite different from conventional ones, there can be produced a single-oriented silicon steel sheet in which the parallelism between the rolling direction and the [001] direction of the crystallization grains is very favorable and in which therefore the magnetic induction is very high. As shown in FIGURE 1, the product A obtained by the present invention is superior in the excitation characteristics specifically at a magnetic induction above 15,000 gauss to the conventional single-oriented silicon steel sheet B.

The present invention shall now be explained in detail in the following.

The silicon steel material which is a starting material in the present invention means an ingot made by solidifying by any casting method a molten steel made by such a steel making method which is an already known art as, for example, by an open-hearth furnace, electric furnace or converter or melted by such a known melting method as, for example, by a high frequency electric furnace or vacuum melting furnace. A slabby ingot obtained by a continuous casting method, which recently came into wide use, can be also used as a material in the present invention. The atmosphere in the case of casting is usually of air but may be vacuum or of an inert gas as well.

As described above, the material in the present invention may be made by any steel making, melting and casting methods. But the composition of the material must satisfy the following conditions, irrespective of the method for producing the same. The material (which shall be known as the ingot hereinafter) must contain 0.025 to 0.085% C, 2.5 to 4.0% Si, 0.010 to 0.065% acid-soluble Al and 0.005 to 0.050% S, the rest being iron and mixed impurities. The acid-soluble Al so called here designates Al soluble in a dilute sulphuric acid solution of 1 part of sulphuric acid to 9 parts of water and is, to be concrete, a total of Al in a solid-solution in the silicon steel and such nitride of Al as AlN. The acid-insoluble Al means such Al oxide as  $Al_2O_3$ . It is needless to say that the sum total of acid-soluble Al and acid-insoluble Al is total Al.

As described above, the present invention is characterized by the steps of hot-rolling a silicon steel ingot of specified contents of C, Si, acid-soluble Al and S so as to be a hot-rolled sheet, cold-rolling the above mentioned hot-rolled sheet at a reduction in thickness of 5 to 40%, thereafter annealing the cold-rolled sheet at such high temperature as 950 to 1200° C. so that AlN having such a size as will markedly facilitate the production of secondary recrystallization grains of the (110)[001] orientation may be precipitated, cold-rolling the annealed sheet at a reduction in thickness of 81 to 95% and subjecting the thus obtained sheet to known annealings for decarburization and secondary recrystallization.

That is to say, if the contents of C, Si, acid-soluble Al and S in the silicon steel ingot are specified as in the present invention and the annealing before the final cold-rolling is carried out at such high temperature as 950 to 1200° C. for 30 seconds to 30 minutes, AlN having such a size as can produce secondary recrystallization grains of the (110)[001] orientation in which the parallelism between the <100> axis and the rolling direction is very excellent will be able to be precipitated as more than 0.0020% N as AlN. Only in case such a steel sheet is finally cold-rolled at such a high reduction in thickness as is specified in the present invention, the object of the present invention will be able to be attained. In case any one of the elements of the composition deviates from the specified range or in case the temperature and time of the final annealing do not conform to the specified conditions, it will be impossible to precipitate the specified amount of

AlN having such a size as will produce secondary recrystallization grains of the (110)[001] orientation in the steel sheet before the final cold-rolling, whereby the object product will not be obtained.

As in the above, in the present invention, the three conditions of the composition, the annealing carried out just before the final cold-rolling and the final cold-rolling are closely related with one another. By the treating steps having such three conditions, there can be obtained a product far superior in magnetic characteristics to any conventional single-oriented silicon steel sheet.

The reasons for specifying the composition of the ingot in the present invention shall be explained in the following.

A silicon steel ingot which contained about 3% Si and 0.040% C and in which the contents of acid-soluble Al and S varied as shown in FIGURE 2 was rolled while hot to be a hot-rolled sheet 3 mm. thick. The content of C in the hot-rolled sheet was 0.040%. The sheet was first cold-rolled at a reduction in thickness of 30%, was then annealed at 1100° C. for 5 minutes, was finally cold-rolled at a reduction in thickness of 85.7% to be of a final gauge of 0.3 mm., was then decarburized at 800° C. and was finally box-annealed at 1200° C. The relation between the magnetic induction  $B_{10}$  of the thus obtained product and the acid-soluble Al and S in the ingot is shown in FIGURE 2. That is to say, the magnetic induction  $B_{10}$  of the final product obtained by the producing steps according to the present invention is greatly different depending on the contents of S and acid-soluble Al. As evident from this diagram, the object product of the present invention in which the magnetic induction  $B_{10}$  in the rolling direction is higher than 18,000 gauss will be obtained when the acid-soluble Al is 0.010 to 0.065% and S is 0.005 to 0.050%. As shown by the curve of the magnetic induction  $B_{10}$  in FIG. 2 the addition effect of S and acid-soluble Al is determined by the following formula of the addition ratio of both components:

$$\frac{S(\%)}{\text{acid-soluble Al}(\%) + \alpha} = 0.8$$

In this formula  $\alpha$  is to be made the value ranging from 0.025 (straight line A in FIG. 2) to -0.015 (straight line B in FIG. 2). It is most preferable to contain S and acid-soluble Al in such a ratio that  $\alpha$  may be about 0.010 (straight line C in FIG. 2) in the above formula, when S amounts to 0.020 to 0.040% and acid-soluble Al 0.020 to 0.040%. It was shown that in this case the magnetic induction  $B_{10}$  of the final product exceeds 19,000 gauss. However, if S is less than 0.005% or more than 0.050% and acid-soluble Al is less than 0.010% or more than 0.050%, the production of secondary recrystallization grains of the (100)[001] orientation in the final annealing will become remarkably low and the magnetic induction  $B_{10}$  in the rolling direction of the final product will not exceed 18,000 gauss, even if the addition ratio of S and acid-soluble Al would be limited in the range as mentioned in the above formula. For the above described reasons, the composition of the silicon steel ingot to be used in the present invention should be so specified that S be in the range of 0.005 to 0.050%, acid-soluble Al in the range of 0.010 to 0.050% and moreover in the addition ratio of both components of

$$\frac{S(\%)}{\text{acid-soluble Al}(\%) + \alpha} = 0.8$$

$\alpha$  be in the range of 0.025 to -0.015.

Si is specified to be in the range of 2.5 to 4%. In case it is less than 2.5%, there will be a disadvantage that the electric resistance will be so low and the eddy current loss will be so high that the core loss value will be high. On the contrary, in case Si is more than 4%, breaks due to brittleness will be caused in cold-rolling. Therefore, in the present invention, the content of silicon in the silicon steel ingot is defined to be 2.5 to 4%.

However, as seen in FIGURE 2, even if a silicon steel ingot in which Si, acid-soluble Al and S are in the above mentioned specified ranges is treated, the magnetic induction  $B_{10}$  of the final product will not exceed 18,000 gausses in some case. Taking such a case into consideration, a further condition of composition must be specified. It is the content of aluminium nitride or AlN. This AlN must be precipitated in the steel sheet before the final cold-rolling but need not always be precipitated in the ingot, because, if the ingot contains Al, the Al will react with N in the steel in the heat-treatment and will be precipitated as AlN in the steel. FIGURE 2 shows also a specification of such content of AlN in the steel sheet before the final cold-rolling as is required in the present invention. The numeral attached to each point in the diagram represents the content of AlN in the steel sheet before the final cold-rolling in N as AlN in

percent by weight  $\times 10^4$

As seen from this, in case N as AlN is less than 0.0020%, even if the main elements Si, acid-soluble Al and S in the above mentioned ingot are in the specified ranges, the magnetic induction  $B_{10}$  in the rolling direction of the final product will not exceed 18,000 gausses and the object of the present invention will not be able to be attained.

For the above reasons, the content of AlN in the steel sheet before the final cold-rolling in the present invention must be such that N as AlN is more than 0.0020%.

Now, it has been found to be requisite that AlN having such a size as being able to produce secondary recrystallization grains of the (110)[001] orientation should be present in the steel sheet before the final cold-rolling, and that such AlN should be precipitated in the annealing step just before the final cold-rolling. The precipitation of such AlN can be attained by adjusting the content of C in the steel sheet before the annealing so as to be at least 0.020 to 0.080% and annealing the steel sheet at 950 to 1200° C. for 30 seconds to 30 minutes. It has been confirmed that, in case the content of C in the steel sheet before the annealing is less than 0.020% or exceeds 0.080%, even if the content of AlN is such that N as AlN is more than 0.0020%, the precipitate size will not be proper and, as a result, secondary recrystallization grains of the (110)[001] orientation will not be produced in the final annealing. Therefore, in the present invention, in order to adjust the content of C in the steel sheet before the annealing so as to be in the range of 0.020 to 0.080%, it is necessary that the silicon steel ingot should contain at least 0.025 to 0.085% C, because slight decarburization (of about 0.005%) will occur in the hot-rolling of ingot and subsequent annealing of the ingot.

As described above, it has been confirmed that in the present invention, the contents of the four elements in the silicon steel ingot should be so defined as to be 0.025 to 0.085% C, 2.5 to 4.0% Si, 0.010 to 0.065% acid-soluble Al and 0.005 to 0.050% S and that the C content in the steel before the annealing step immediately antecedent to the final cold-rolling should be adjusted to be in the range of 0.020 to 0.080% in order that AlN having such a size as will produce secondary recrystallization grains of the (110)[001] orientation may be precipitated in an amount of at least 0.0020% of N as AlN in said annealing step. Only when such specifications of the composition and the final cold-rolling step at such a high reduction in thickness as is described in the following are closely combined together, it will be possible to produce a single-oriented silicon steel sheet of a high magnetic induction.

The concrete steps of one embodiment of the method according to the present invention are carried out in the following sequence. After the hot-rolled silicon steel sheet is pickled, it is subjected to a cold-rolling, the cold-rolled sheet is annealed and the annealed sheet is again subjected to a cold-rolling by the conventional two annealing steps, that is, the annealing for decarburization and that for producing recrystallization grains to obtain a de-

sired final product. Hereinafter the first cold-rolling will be designated as the first cold-rolling step, the sequent annealing as the intermediate annealing step, the following cold-rolling as the final cold-rolling step and the annealing for producing recrystallization grains as the final annealing. Of course, each cold-rolling step may comprise several rolling passes. However, in the present invention the cold-rolling step prior to the final cold-rolling step is not limited to only one. It may be repeated even several times, combined with the sequent annealing step according to conditions. Further, in another embodiment even the first cold-rolling step may be omitted. In such a case the cold-rolling will be carried out only in one step (that is, the final cold-rolling step as designated here) after the antecedent annealing step. The features of the present invention reside in the reduction in thickness in the cold-rolling steps, particularly in the final cold-rolling step and the annealing conditions in the intermediate annealing step immediately prior to the final cold-rolling step.

First of all, the cold-rolling condition will be explained.

Silicon steel ingots made by melting in an electric furnace and casting and containing 0.040% C, 3.02% Si, 0.031% acid soluble Al and 0.030% S were bloomed, hot-rolled and finished to be hot-rolled sheets 7.0, 5.0, 3.4, 3.0, 2.6 and 1.8 mm. thick. The content of C in each hot-rolled sheet was about 0.040%. By using each sheet as a starting material, the first cold-rolling step was carried out at a reduction in thickness of 0 to 80% as shown in the lower part in FIGURE 3. (In this case, 0 was not subjected to the first cold-rolling step and was therefore subjected to only one final cold-rolling step.) The sheet was then annealed at 1100° C. for 5 minutes, was then subjected to the second cold-rolling step (final cold-rolling step) at the reduction in thickness also shown in the lower part of the diagram so as to be of a final thickness of 0.3 mm., was decarburized in wet hydrogen at 800° C. for 5 minutes and was finally box-annealed at 1200° C. for 20 hours. The relation between the magnetic induction  $B_{10}$  of the thus obtained product and the reduction in thickness is shown in FIGURE 3. The facts evident from this diagram are the following two points. It has been found that the reduction in thickness in the final cold-rolling step required for the magnetic induction  $B_{10}$  in the rolling direction of the product to exceed 18,000 gausses should be at least 81%, but not exceed 95% and is most preferably in the range of 83 to 92% and that the reduction in thickness in the first cold-rolling step should be kept less than 40%. However, in case the first cold-rolling step is carried out at a reduction in thickness not exceeding 5%, the effect on the improvement of the magnetic characteristics of the product will not be more remarkable than in the later described case of making the final product thickness in only one cold-rolling step, that is, in the case of omitting the first cold-rolling step. Thus, in such a case it will be meaningless to carry out the cold-rolling in two steps, which means that the reduction in thickness in the first cold-rolling step should be in the range of 5 to 40%.

To sum up, the cold-rolling may be carried out only in one step or in two steps or even in several steps. In case the cold-rolling is carried out only in one step, the reduction in thickness should be 81 to 95%. But, in case it is carried out in two or more steps, the following conditions must be absolutely fulfilled: that is, the final cold-rolling step should be carried out at a reduction in thickness of 81 to 95% and any cold-rolling step prior to the final cold-rolling step at a reduction in thickness of 5 to 40%. The cold-rolling treatments at such specific reduction in thickness have never been seen in any already disclosed process for producing single-oriented silicon steel sheets. Only in the case of using a silicon steel ingot of the above specified composition contents, such cold-rolling treatments will be significant.

The silicon steel sheet to be used as an iron core for

electric devices is mostly about 0.3 mm. thick. When such a final sheet thickness is to be obtained with two cold-rolling steps and one annealing step, it will be most preferable that the thickness of the hot-rolled sheet is 2.6 to 3.4 mm. However, in case the thickness of the hot-rolled sheet is 7 mm. a product high in magnetic induction will be hardly obtained with two cold-rolling steps only. In such a case, the cold-rolling at a reduction in thickness of 5 to 40% and the annealing are repeated several times, followed by the final intermediate annealing and the final cold-rolling to obtain a product of a high magnetic induction comparable to that of the former.

In the present invention, irrespective of the sheet thickness of the final product, a product high in magnetic induction may be obtained. However, usually, if the thickness of the hot-rolled sheet is more than 7 mm., it is difficult to wind the sheet to be in the form of a coil or to strip and cold-roll it. Further, it is difficult in the hot-rolling technique to make a hot-rolled sheet less than 1.5 mm. thick. Therefore, for factory conditions, it is defined that in case two or more cold-rolling steps are included the sheet thickness should be 1.5 to 7 mm.

Though the theoretical ground of the cold-rolling treatment in the present invention is not apparent, a clear difference from any conventional cold-rolling treatment can be perceived from the observation of the crystal orientation. FIGURES 4 and 5 show with (110) and (100) pole figures the crystal orientations obtained after carrying out the respective annealing in the products corresponding to A (of  $B_{10}$  of 19,100 gauss) and B (of  $B_{10}$  of 17,600 gauss) in FIGURE 3, respectively.

From the above figures it is evident that the crystal orientation shown after carrying out the decarburization annealing is quite different between the case of carrying out the cold-rolling treatments (at reduction in thickness of 20% in the first cold-rolling step and 87.5% in the final cold-rolling step) according to the present invention and the case of carrying out the conventional cold-rolling treatments (at reduction in thickness of 70% in the first cold-rolling step and 66.7% in the final cold-rolling step).

FIGURES 4 1 and 5 1 are (110) pole figures after the respective intermediate annealings (at 1100° C. for 5 minutes in the former and at 1100° C. for 5 minutes in the latter). FIGURES 4 2 and 5 2 are (110) pole figures after the decarburizing annealings (at 850° C. for 5 minutes in both). FIGURES 4 3 and 5 3 are (100) pole figures after the final annealings (at 1200° C. for 20 hours in both). The numerals in FIG. 4 1 and 2, and FIG. 5 1 and 2 designate the strength of crystal orientation as compared with that of random crystal orientation in the X-ray diffraction as the standard value, taking the latter as 1.0 and those in FIG. 4 3 and FIG. 5 3 the grain numbers of the secondary recrystallization grains.

As described later, the decarburizing annealing is carried out to remove C detrimental to the development of secondary recrystallization grains of the (110)[001] orientation in the final annealing and at the same time to make the cold-rolled structure a primary recrystallization structure. The primary recrystallization orientation (FIGURE 5 2) after the decarburizing annealing in the case of carrying out the conventional cold-rolling treatment is a main orientation rotated by about  $\pm 25$  degrees around the <110> rotation axis parallel with the rolling direction with the (100)[001] orientation as a center. On the other hand, the crystal orientation (FIGURE 4 2) after the decarburizing annealing in the case of carrying out the cold-rolling treatment according to the present invention has a feature that the <110> rotation axis is deviated by about 20 to 25 degrees to right and left from the rolling direction. The parallelisms between the <100> axis of the secondary recrystallization grains of the (100)[001] orientation produced when both of them were finally annealed and the rolling direction are as respectively shown by (100) pole figures in FIGURES 4 3 and 5 3. The former is remarkably superior in the

parallelism and is higher in magnetic induction  $B_{10}$ . It is needless to say that the production of such secondary recrystallization grains arranged in direction is possible only by subjecting a hot rolled silicon steel sheet of such composition as is specified in the present invention to the above mentioned cold rolling treatment.

It is also possible to subject the hot rolled sheet to an annealing at temperatures of 950 to 1200° C. as above mentioned, then cold-roll one time the thus annealed sheet at a reduction in thickness of 83 to 96% as shown in FIG. 3 and thereafter subject the thus obtained sheet to known annealings for decarburization and secondary recrystallization. However, in this case the thickness of the hot-rolled sheet must be 1.5 to 5 mm.

The annealing step shall now be described. First of all, the conditions of the intermediate annealing step immediately prior to the final cold-rolling step, which make one of the most important features in the present invention, shall be described. A silicon steel ingot prepared by melting in an electric furnace and casting and containing 0.038% C, 3.0% Si, 0.030% acid-soluble Al and 0.028% S was bloomed and hot-rolled to be a hot-rolled sheet having a thickness of 3.0 mm. The content of C in the hot-rolled sheet was 0.037%. The sheet was cold-rolled by 30%, was then annealed in  $H_2$  at temperatures of 800, 900, 950, 1000, 1050, 1100, 1150, 1200 and 1300° C. for 5 minutes each, was then finally cold-rolled at a reduction in thickness of 85.7% to be of a product thickness, was annealed to be decarburized at 800° C. for 5 minutes and was then finally annealed in  $H_2$  at 1200° C. for 20 hours. The relation between the magnetic induction  $B_{10}$  in the rolling direction of the product and the annealing condition before the final cold-rolling is shown in FIGURE 6.

It is understood from this that the annealing temperature to obtain a product of a magnetic induction  $B_{10}$  of 18,000 gauss in the rolling direction as desired in the present invention must be in the range of 950 to 1200° C. and that the most preferable temperature range is 1050 to 1150° C. The annealing time in this temperature range must be such that the time for which the steel sheet is kept at such temperature is at least 30 seconds to 30 minutes. If the time is less than 30 seconds, it will be impossible to precipitate the specified amount of AlN of such a size is required for the steel sheet, while in case the time exceeds 30 minutes, the crystal grains will grow, after the recrystallization has been completed, resulting in an incomplete development of the secondary recrystallization grains of the (110)[001] orientation in the final annealing in both cases. As already described, the atmosphere for the annealing has nothing to do with the precipitation of AlN in the steel sheet before the final cold-rolling step. Usually, in case the silicon steel ingot is made in an open-hearth furnace or the like, the ingot as it is will contain more than 0.0040% N which will further increase in the hot-rolling. Therefore, AlN having the desirable size will be able to be precipitated as more than 0.0020% N as AlN by subjecting the steel sheet to the intermediate annealing immediately prior to the final cold-rolling step, even if nitrogen is not specifically added in this annealing, provided that the content of C in the steel sheet is being kept in the range of 0.020 to 0.080% as already specified. Hence, any of reductive and neutral atmospheres such as, for example, of  $H_2$ , Ar and  $N_2$  gases or mixtures of them may be used for the atmosphere for the annealing. However, in case the silicon steel ingot is made by melting in a vacuum melting furnace or the like or by casting by a vacuum casting method or the like, N in the ingot will be so little that, unless nitrogen is added in the annealing before the final cold-rolling, it will be impossible to precipitate more than 0.0020% N as AlN. The method of adding nitrogen is not specified. But, in the present invention, it is recommended to carry out the annealing in a neutral or reductive gas containing at least 10% by

volume  $N_2$ . The reason why the annealing immediately prior to the final cold-rolling step in the present invention is carried out at a temperature higher than in the annealing in any conventional process for producing single-oriented silicon steel sheets is presumed to be that, on account of C contained in the steel sheet before being subjected to the annealing the  $\alpha$ - $\gamma$  transformation will occur in this range of annealing temperature and the precipitation of AlN having such a size as will facilitate the production of secondary recrystallization grains of the (110)[001] orientation will be accelerated thereby. It is considered that such AlN together with the subsequent final cold-rolling treatment at a high reduction in thickness and annealing treatment will make it possible to produce nuclear crystal grains of the (110)[001] orientation very excellent in the parallelism between the  $<100>$  axis and the rolling direction. In case the intermediate annealing is to be repeated between several cold-rolling steps before the final intermediate annealing, it may be carried out at such temperature and for such time as are sufficient to make the cold-rolled structure (obtained by cold-rolling) a primary recrystallization structure.

The steel sheet finally cold-rolled to be of a product sheet thickness is then subjected to the carburizing annealing. This annealing is to make the cold-rolled structure a primary recrystallization structure and at the same time to remove C detrimental to the development of secondary recrystallization grains of the (110)[001] orientation in the final annealing. For the decarburizing method may be used any known method. For example, there can be enumerated a method of annealing in wet hydrogen at a temperature of 750 to 850° C. for a short time.

The final annealing should be carried out at such temperature and for such time that secondary recrystallization grains of the (110)[001] orientation can well develop. In order that the secondary recrystallization grains may perfectly develop, the steel sheet must be annealed at a temperature higher than 1000° C. for at least 5 hours. Even if the atmosphere for the final annealing is a neutral or reductive atmosphere or such weakly oxidative atmosphere as will not remarkably oxidize the steel sheet, the object product of the present invention in which the magnetic induction  $B_{10}$  in the rolling direction is more than 18,000 gauss will be obtained. However, in order to reduce the core loss value, it is usually recommended to finally anneal the steel sheet in  $H_2$ .

#### Example 1

A silicon steel ingot containing 0.037% C, 3.00% Si, 0.028% acid-soluble Al and 0.031% S was prepared in an electric furnace, was bloomed and was hot-rolled to be a hot-rolled sheet 3 mm. thick. The content of C in the hot-rolled sheet was 0.036%. The sheet was first cold-rolled by 30% and was then annealed in  $H_2$  at 1100° C. for 5 minutes.

The content of AlN in the steel sheet after the annealing was 0.0049% N as AlN. The sheet was then cold-rolled by 85.7% to be of a product sheet thickness of 0.3 mm., was decarburized in wet hydrogen at 800° C. for 5 minutes, was pickled and was finally annealed in hydrogen at 1200° C. for 20 hours.

The magnetic characteristics in the rolling direction of the product were as follows:

$B_{10}=19,070$  gauss

W 15/50 (core loss value at 15,000 gauss at 50 cycles) = 0.99 watts/kg.

W 17/50 (core loss value at 17,000 gauss at 50 cycles) = 1.30 watts/kg.

Thus a very excellent single-oriented silicon steel sheet was obtained.

#### Example 2

5 A silicon steel ingot containing 0.035% C, 3.00% Si, 0.037% acid-soluble Al and 0.036% S was prepared in an electric furnace, was bloomed and was hot-rolled to be a hot-rolled sheet 5 mm. thick. The sheet was cold-rolled by 30%, was annealed at 900° C. for 2 minutes so as to be recrystallized and was then again cold-rolled by 30%. At this time, the content of C in the steel sheet was 0.031%. The sheet was then annealed in  $H_2$  at 1100° C. for 5 minutes. The content of AlN in the steel sheet after the annealing was 0.0046% N as AlN.

10 The sheet was then cold-rolled by 87.8% to be of a product sheet thickness of 0.3 mm., was decarburized in wet hydrogen at 800° C. for 5 minutes and was finally annealed in  $H_2$  at 1200° C. for 20 hours. The magnetic characteristics in the rolling direction of the product were as follows:

20  $B_{10}=19,000$  gauss

W 15/50=1.01 watts/kg.

W 17/50=1.31 watts/kg.

#### Example 3

25 A silicon steel ingot containing 0.040% C, 3.02% Si, 0.030% acid-soluble Al and 0.030% S was prepared in an electric furnace, was bloomed and was hot-rolled to be a hot-rolled sheet 3 mm. thick. The content of C in the hot-rolled sheet was 0.040%. It was annealed in  $H_2$  at 1050° C. for 5 minutes.

30 The content of AlN in the steel sheet after the annealing was 0.0055% N as AlN. The sheet was then cold-rolled at a reduction in thickness of 89% to be of a product sheet thickness of 0.33 mm., was decarburized in wet hydrogen at 800° C. for 5 minutes and was finally annealed in hydrogen at 1200° C. for 20 hours.

35 The magnetic characteristics in the rolling direction of the product were as follows:

40  $B_{10}=18,800$  gauss

W 15/50 (core loss value at 15,000 gauss at 50 cycles)=1.05 watts/kg.

45 W 17/50 (core loss value at 17,000 gauss at 50 cycles)=1.35 watts/kg.

What is claimed is:

45 1. A process for producing single-oriented silicon steel sheet of (110)[001] orientation, in which a silicon steel ingot composed of 0.025 to 0.085 wt. percent C, 2.5 to 4.0 wt. percent Si, 0.010 to 0.050 wt. percent acid-soluble Al and 0.005 to 0.050 wt. percent S and the rest being iron is hot-rolled to produce a hot-rolled steel sheet, said hot-rolled steel sheet is subjected to an annealing and cold-rolling to obtain a steel sheet of final thickness, said steel sheet of final thickness is thereafter subjected to an annealing for decarburization and further for secondary recrystallization, comprising the steps of hot-rolling a material, in which the ratio of S and acid-soluble Al is made to be

50 55  $\frac{S(\%)}{\text{acid-soluble Al}(\%)} + 0.025 \text{ to } -0.015 = 0.8$

60 to make the thickness of said material to 1.5 mm. to 7 mm., cold-rolling the thus hot-rolled steel sheet at a reduction in thickness of 5 to 40%, annealing the cold-rolled sheet at a temperature ranging from 950 to 1200° C. for 30 seconds to 30 minutes and then finally cold-rolling the thus annealed steel sheet at a reduction in thickness of 81 to 95%.

65 2. A process for producing single-oriented silicon steel sheet claimed in claim 1, in which a material, in which the ratio of S and acid-soluble Al is made to be

70  $\frac{S(\%)}{\text{acid-soluble Al}(\%)} + 0.010 = 0.8$   
is subjected to a hot-rolling.

75 3. A process for producing single-oriented silicon steel

11

sheet claimed in claim 1, in which a cold-rolled steel sheet containing 0.020 to 0.080 wt. percent C is annealed at a temperature ranging from 950 to 1200° C. for 30 seconds to 30 minutes and thereafter the thus annealed steel sheet is finally cold-rolled.

4. A process for producing single-oriented silicon steel sheet claimed in claim 1, in which a material is hot-rolled to make the thickness of said material to 1.5 to 7 mm., the thus obtained steel sheet is then annealed at a tempera-

5

12

ture ranging from 950 to 1200° C. for 30 seconds to 30 minutes and the thus annealed steel sheet is cold-rolled at a reduction in thickness of 83 to 96%.

No references cited.

DAVID L. RECK, *Primary Examiner.*

N. F. MARKVA, *Assistant Examiner.*